

# UNITED STATES PATENT OFFICE.

FRANK S. LOW, OF NEW YORK, N. Y., ASSIGNOR TO THE CUTLER-HAMMER MFG. CO., OF MILWAUKEE, WISCONSIN, A CORPORATION OF WISCONSIN.

## MATRIX-MAT.

1,265,796.

Specification of Letters Patent. Patented May 14, 1918.

No Drawing.

Application filed June 25, 1914. Serial No. 847,318

*To all whom it may concern:*

Be it known that I, FRANK S. Low, a citizen of the United States, residing at New York, in the county of New York and State of New York, have invented new and useful Improvements in Matrix-Mats, of which the following is a full, clear, concise, and exact description.

My invention relates to matrix mats. 10 These mats are employed in the art of stereotype printing to take an impression of the set type and thus produce a matrix from which a stereotype plate may be cast.

The practice is to place a mat upon the set 15 type and then apply pressure until the mat receives an impression. This mat then becomes a matrix from which a stereotype plate may be cast. It is usually required that a stereotype plate be semi-cylindrical 20 in form. The matrix when taken from the type is flat and in consequence it must be capable of being bent into semi-cylindrical form when it is placed in the casting machine.

25 It is manifest that the mat must be capable of receiving an impression and then holding this impression while a stereotype plate is being cast. Often it is required that many plates be cast from the same matrix.

30 The two principal mats which have been developed are wet mats and dry mats.

Wet mats are made up of sheets of paper which are bound together and impregnated with plastic paste. Starch paste has been 35 employed extensively.

It requires considerable labor and skill to produce a wet mat such as has heretofore been successful. The operator first coats a sheet of paper with the starch paste; then he 40 places a second sheet over this paste and covers the second sheet with starch paste, and so on until the sheets have been multiplied to produce a mat of the required thickness. It is required that this mat be kept in 45 a moist condition and not allowed to dry until it is used; otherwise the starch paste will not be sufficiently plastic to produce a successful matrix. It is difficult to keep a wet mat in proper condition for molding 50 and furthermore delay, trouble and expense are experienced in drying the mat after it is molded so that a stereotype plate may be recast.

It is obvious that the starch must be sufficiently plastic to readily receive the impres-

sion and then must be capable of becoming hard or setting so that the impression will be maintained and withstand the pressure of the molten metal in casting the stereotype plate. The paste is usually set by subjecting 60 it to heat while the mat is still on the type. After the paste is set the mat must still be sufficiently flexible to allow it to be readily bent and manipulated. It must be substantially non-shrinkable so as not to distort or 65 destroy the impression, or alter the predetermined dimensions of the printed page.

Where there are large open spaces between the type, bolsters are produced in the mat. If the bolsters are more than a certain 70 size paper pieces must be put back of them so that they will stand up and this involves considerable labor and loss of time.

Anything which contributes to producing 75 a matrix rapidly is important in this art.

Wet mats have the property of plastic material, and hence actually mold the impression. This gives the best results in the matrix. The surface is smooth and dense and the impression sharp, clear and deep. 80

The dry mats which have been developed do not really have plastic characteristics. In other words, their material does not actually mold in receiving an impression. The material in fact is of such character that if one 85 particle thereof is segregated from another it will not again integrally re-unite. What actually happens in making an impression is that the mat is embossed or stamped. The character of the material is such that a deep 90 impression cannot be obtained.

If the stereotype plate sticks to the mat it destroys the matrix. The face of the matrix must be very dense, compact and smooth without any fissures, disruptions or fractures 95 even though they be merely microscopic, as the molten metal under pressure will creep in to even the slightest crevice or flow around the slightest ledge and cause the matrix to stick. Even minute fibers lying on the surface or forming the slightest crevices may cause the stereotype plate to stick. 100

The dry mats have the advantage over the wet mats in that they preserve their properties of taking an impression indefinitely, 105 and hence they may be expeditiously manufactured in quantities and stored until required for use.

Wet mats will give a deep clear impression and be absolutely smooth, but it takes 110

a long time to dry them, and their plasticity cannot be preserved without great inconvenience and trouble. Dry mats will remain in an operative condition, but will not allow 5 a deep impression. Cracks, fissures and disruptions are very likely to be produced in making the impression, and moreover, their face is not sufficiently smooth to produce the best results.

10 The object of the present invention is to produce a mat which will be plastic and which will normally maintain this property indefinitely.

In accordance with this invention, a suitable sheet, as for instance, paper, has incorporated therewith a plastic material which will preserve its plasticity so long as it is subjected to moisture, and to maintain sufficient moisture there is incorporated with 15 the plastic material a hygroscopic material. The mat thus obtained fundamentally consists of fibrous material and hygroscopic plastic material, and these things are combined in such a way and are of such character that the mat will not only normally preserve its moldable properties indefinitely, but will withstand the heat to which it must be subjected. Matrices produced from these 20 mats have strength, flexibility, sharp, clear 25 and deep impressions, smooth and dense surfaces and are devoid of fissures, ledges or crevices.

One way in which the invention has so far been carried out will now be explained.

30 A thick sheet of fibrous absorptive paper is impregnated with a solution of hygroscopic starchy material. This solution must be thin and limpid in order to penetrate the paper. Ordinary unmodified starch will not 35 produce a sufficiently thin and limpid solution. To obtain a solution of the required hygroscopic starchy material, the following method is followed:

15 pounds of soluble or modified starch, 45 2 $\frac{1}{2}$  pounds of magnesium oxid, and 4 $\frac{1}{2}$  pounds of water, are mixed and then 7 $\frac{1}{2}$  pounds of 70 per cent. acetic acid is added to this mixture. The mixture thus obtained is heated to, for instance, 170° F. and 50 50 pounds of water are finally added. This produces a solution which is very thin and limpid, and which will readily impregnate the sheet of paper. The reaction of the magnesium oxid with the acetic acid produces 55 magnesium acetate which is hygroscopic. It has been found that the solution acts very satisfactorily between 120° and 140° F. The thick sheet of paper is now saturated or impregnated with the impregnating solution.

60 The thick sheet has a rather irregular coarse surface, so it is found preferable to provide it with a facing of finer texture so as to obtain a surface that will be very 65 smooth and also impervious to molten stere-

otype metal. The facing may be made up of a thinner and finer sheet of fibrous absorptive paper, and one or more sheets of tissue or onion skin paper, the tissue or onion skin paper constituting the face of the 70 mat. These sheets are all pasted one upon another by means of a starchy paste, which is made up of three mixtures:

First: 1 $\frac{1}{2}$  pounds cassava starch, 1 $\frac{1}{2}$  gallons of water;

Second:  $\frac{1}{16}$  pound magnesium oxid,  $\frac{5}{2}$  gallon water,  $\frac{3}{2}$  gallon 70 per cent. acetic acid:

Third:  $\frac{1}{4}$  gallon gum arabic solution made up of 1 pound gum to  $\frac{1}{4}$  gallon water.

These three mixtures are combined and heated to 160° or more F.

Blanc fixe clay whiting or the like may be put into the paste to facilitate the production of a smooth face.

Of course various modified starches may be employed in the impregnating solution, the purpose being to obtain a starch which will produce a sufficiently thin and limpid solution to impregnate the paper.

This mat may be expeditiously manufactured by means of a machine in which there is a roll of thick paper, a roll of thin paper, and one or more rolls of tissue paper. The thick paper first passes through the impregnating solution and then the thin paper is pasted thereon. Finally the tissue paper is pasted to the thin paper. The web produced is passed through a drier wherein the excess water is removed, and then it is cut into 100 mats of the required size.

Of course the various proportions and the specific materials herein enumerated to set forth an embodiment of my invention may be modified in various ways and the process 105 and method of combining them may be varied without departing from my invention.

Having thus described my invention, what I claim as new and desire to secure by Letters Patent is,

1. A matrix mat consisting of fibrous material and a hygroscopic plastic material which will not be decomposed by the heat to which it is subjected.

2. A matrix mat consisting of fibrous material and hygroscopic starchy material which will not be decomposed by the heat to which it is subjected.

3. A matrix mat having a sheet of fibrous absorptive paper impregnated with a solution of hygroscopic plastic material which will not be decomposed by the heat of the molten metal.

4. A matrix mat having a sheet of fibrous absorptive paper impregnated with a solution of hygroscopic starchy material which will set when moisture is removed therefrom and which will not be decomposed by the heat to which it is subjected.

5. A matrix mat having a sheet of fibrous absorptive paper impregnated with modified starch and hygroscopic material which will not be decomposed by the heat to which it is subjected.

6. A matrix mat having a sheet of fibrous absorptive paper containing starch and hygroscopic material, the hygroscopic material being of such character as will not be 10 decomposed by the heat to which the mat is subjected.

7. A matrix mat having a sheet of fibrous absorptive paper impregnated with hygroscopic plastic material which will not be 15 decomposed by the heat to which it is subjected and a facing pasted thereon.

8. A matrix mat having a sheet of fibrous absorptive paper impregnated with modified starch containing hygroscopic material 20 which will not be decomposed by the heat to which it is subjected.

9. A matrix mat having a sheet of fibrous absorptive paper impregnated with modified starch containing hygroscopic material and 25 a facing fixed thereon by paste made up from ordinary starch and hygroscopic material.

10. A matrix mat having a sheet of fibrous absorptive paper containing modified starch 30 and a hygroscopic material which will not be decomposed by the heat to which it is subjected.

11. A matrix mat having a sheet of fibrous absorptive paper containing modified starch and magnesium acetate.

12. A matrix mat comprising a composite sheet containing hygroscopic plastic material which will not be decomposed by the heat to which it is subjected.

13. A matrix mat comprising a composite

sheet containing hygroscopic starchy material which will not be decomposed by the heat to which it is subjected.

14. A matrix mat comprising a composite sheet containing modified starch and a 45 hygroscopic material which will not be decomposed by the heat to which it is subjected.

15. A matrix mat comprising a composite sheet containing modified starch and mag- 50 nesium acetate.

16. A matrix mat having a sheet of fibrous absorptive material impregnated with a solution containing modified starch and magnesium acetate.

17. A matrix mat having a sheet of fibrous absorptive material containing modified starch and magnesium acetate and a facing of tissue paper affixed thereto by means of a paste containing ordinary starch and 60 magnesium acetate.

18. A matrix mat comprising a sheet of fibrous material impregnated with a modified starch and a compound formed from magnesium oxid and acetic acid.

19. A matrix mat consisting of fibrous material and a hygroscopic plastic material which will not be affected by the heat to which it is subjected in use.

20. A matrix mat consisting of fibrous material and hygroscopic starchy material which will not be affected by the heat to which it is subjected in use.

In witness whereof, I have hereunto subscribed my name in the presence of two wit- 75 nesses.

FRANK S. LOW.

Witnesses:

EDWIN B. H. TOWER, Jr.,  
J. E. HUTCHINSON, Jr.

Copies of this patent may be obtained for five cents each, by addressing the "Commissioner of Patents.  
Washington, D. C."